

Patented May 15, 1928.

1,669,490

# UNITED STATES PATENT OFFICE.

WALLACE SAVAGE, OF NEW YORK, N. Y., ASSIGNOR TO SAVAGE-RUBBER CORPORATION, A CORPORATION OF NEW JERSEY.

## VULCANIZED PITCHES.

No Drawing.

Application filed January 17, 1922. Serial No. 529,963.

This invention relates to the production of soft rubber like vulcanized pitches from the "still bottoms" residues obtained as a by-product in the process of refining fatty acids by distillation. These residues are thick, sticky, brownish black tar like oils having a melting point of from 60° to 100° F. and contain from 15 to 30 per cent free fatty acids, about the same amount of glyceride esters or oils and about 40 per cent resin like polymerized oil hydrocarbons. The so-called fatty acid pitches designated and sold in commerce as cotton seed foots, corn oil, beta oil pitches and the like, are made by the pyrolytic distillation of these oily "still bottoms" residues, a large portion of the free fatty acid content of which is superheated to volatilize and separate a yield of low grade pyro-fatty acid distillate. These destructively distilled pitches may have a melting point of from 100° to 350° F., and penetration of 100-0 mm., at 77° F., according to the extent of pyrolysis they have undergone. They are asphalt-like in most of their physical properties, action, treatment and application, but are dissimilar to asphalt chemically due to their fatty origin.

The present invention has particular reference to the production of improved vulcanized fatty acid pitch products characterized by their ability to more completely, rapidly and spontaneously recover their original size and shape after deformation than any known pitch product familiar to those experienced in the art. The vulcanized pitch herein described is suited for use as a packing material for liquid, vapor or gas tight joint seals, especially in large engineering structures, such as are used in the construction of roads, roofs, tanks, dams, conduits, subways, sewers and the like.

Kerite products comprising vulcanized candle tar, the pitch made from the "still bottoms" residues from distilled stearines, have been known in the arts for more than forty years and were first commercially used and known under the name of Callender's pitch. The same type of products including paint solutions of it were later described in the art. Candle tar, as its name implies, is derived from rigid waxy fats of the type used in the manufacture of stearine candles. It yields a vulcanization product having properties influenced by the characteristics of these fats and therefore having much less

elasticity than the products obtained from residues or pitches derived from oils chemically characterized as unsaturated, or having double bonds.

I have discovered that when soft drying oil "still bottoms" residues from fatty acid refining are vulcanized with more than seven per cent sulphur at from 300 to 400° F., a new highly elastic congealed pitch product, resembling soft rubber in its physical properties, is obtained. If the residue is first partially hardened by pyrolytic treatment, blowing air or steam through its melted mass, or dissolving harder bitumens in it, a firmer body will be obtained in the vulcanized product. The higher the iodine value the softer the product will be due to the action of the double bonds on the texture of the hydrocarbon. When pulled, these products stretch considerably and when released, return directly to their original shape. They give under displacing pressure and recover their form as released. These vulcanized residues are firmer than the vulcanization products made from the oils from which the fatty acids were originally obtained and more closely resemble rubber than the so-called rubber-substitutes or vulcanized oils. The distinctive properties of these vulcanized residues are that they are pliable at 32° F., are self-healing when ruptured and have a melting point of 360° F., when fully congealed and cured. By partially subjecting the residue to any of the hardening processes known in the arts such as pyrolytic distillation, air blowing, blending with previously hardened fatty acid pitches or natural mineral bitumen hardeners, such as grahamite or gilsonite, I have found that all intermediate stages between extremely soft and vulcanite hard rubber like properties can be obtained from the vulcanized residue. Also these various stages of pliancy in the vulcanized product can be obtained by softening a hard pyrolytically distilled fatty acid pitch by blending therewith any flux such as solvent mineral or organic oils, fatty acids or their glycerides to obtain the equivalent physical properties in the alternate manner above cited, prior to vulcanization.

In the process of vulcanization, I have found it convenient to add gradually about two-thirds of the sulphur required for the process with agitation to free the hydrogen

sulphide as formed. Thus a semifinished product that can be stored and transported at any temperature is obtained. The final third of the sulphur can be added and the product finished by heating to 370° F., for a few minutes. At temperatures below 275° F., the rate of vulcanization is so slow that the fully sulphured semi-vulcanized product can be stored ready for finishing by heating above 300° F., at any time. Until about seven per cent of sulphur has been incorporated, no congealment of the oily residue takes place apparently regardless of either thermal, catalytic or time conditions. 15 Amounts of sulphur as high as sixty per cent of the mass of the vulcanized product can be used, the excess of uncombined sulphur forming an inert filler of visible crystalline grains. Free sulphur in excessive 20 amounts gives a product having less desirable properties than an equivalent one having a mineral of a structure superior to the sharp rhombic or prismatic sulphur crystals. Accelerators, such as aniline, thiocarbonilide, zinc oxide or magnesia contribute to the speed of vulcanization and improve the quality of the product. Combined sulphur such as antimony sulphurete, sulphur chloride and equivalent vulcanizing 25 agents give products having peculiar characteristics similar to those obtained by their use with rubber gum. In fact most of the processes and materials of vulcanization and compounding as practiced in the 30 rubber art can be applied to fatty acid residue treatment with success. Fillers such as clays, soapstone, magnesia, ochre, barites, asbestos, cotton linters, mineral wool, paper pulp, ground wood, zinc oxide, gas black, 35 lamp black, glue and formaldehyde, mineral rubbers, rubber gums, rubber substitutes and similar materials may be especially mentioned as giving homologous compounds with fatty acid "still bottoms" residues to 40 those obtained with rubber gums which are familiarly known in the art. The function of fillers is to act as a brake on displacement under stresses. Fiber fillers such as asbestos resist both compression and tension, 45 while powders such as carbon black counteract compressive loads, forming a supporting skeleton structure within the compound. Part of the required sulphur of vulcanization generally called free sulphur in rubber parlance performs an identical function so 50 that the compounding of fillers in a compound is actually substituting this class of material for the inert filler phase of sul-

phur that would be obtained by the use of over ten per cent sulphur in the product. 60

The preferable manufacturing procedure is to heat about 3500 lbs. of fatty acid "still bottoms" residues resulting from the treatment of cottonseed, corn, soya bean, garbage grease or like oils in the manufacture of fatty acids to 300° F., in an autoclave supplied with a suitable agitator. Into the mass there are then incorporated 10 lbs. of thiocarbonilide, 20 lbs. zinc oxide, 250 lbs. of melted sulphur, 400 lbs. of #60 asbestos fibers and 80 lbs. of powdered magnesia. Grahamite may or may not be added in amounts from 100 to 400 lbs. according to the requirements as to hardness. The autoclave is sealed, and the temperature increased to 370° F. When the product has ceased foaming and congealed, it is blown out into forms and worked into shape while plastic. After cooling below 140° F. the congealed product takes a permanent set. It can be cut into boards and other simple shapes after it is cold. The scrap is returned to the next autoclave batch and worked over. If 100 lbs. of the sulphur is held out, it may be added to the product upon cooling to 300° F., and a semi-vulcanized product obtained which will congeal upon heating to 370° F., for a few minutes. 75

While I have described in detail the preferred materials and proportions used in my vulcanized products, it is to be understood that known chemical and physical equivalents of the materials used may be employed, all without departure from the spirit of my invention or the scope of the subjoined claims. 90

Having described my invention, I claim:

1. A soft rubber like composition comprising fatty acid "still bottoms" residue products vulcanized with the aid of an accelerator. 100
2. A soft rubber like composition comprising fatty acid "still bottoms" residue products vulcanized with the aid of thiocarbonilide. 105
3. A soft rubber like composition comprising fatty acid "still bottoms" residue products vulcanized with the aid of thiocarbonilide and zinc oxide.
4. A soft rubber like composition comprising fatty acid "still bottoms" residue products vulcanized with the aid of an organic accelerator. 110

In testimony whereof I affix my signature.

WALLACE SAVAGE.